# EUROPEAN PATENT SPECIFICATION

(11) **EP 0 471 505 B1**
(45) Date of publication and mention of the grant of the patent: **02.10.1996**
(21) Application number: 91307268.2
(22) Date of filing: 07.08.1991
(51) Int. Cl.: C23C 28/00, C23C 4/02, C23C 4/04

(54) **Coated article, its use and method of making the same**
Beschichteter Gegenstand
Objet revêtu, son utilisation et procédé de sa fabrication

(30) Priority: 11.08.1990 GB 9017639
(43) Date of publication of application: 19.02.1992
(73) Proprietor: JOHNSON MATTHEY PUBLIC LIMITED COMPANY, London EC1N 8JP (GB)
(72) Inventor: Coupland, Duncan Roy, High Wycombe, Buckinghamshire HP11 1EA (GB); McCabe, Andrew Robert, Headington, Oxford OX3 7AG (GB)
(74) Representative: Wishart, Ian Carmichael

(56) References cited:
- EP-A- 0 183 638
- WO-A-86/04615
- FR-A- 2 084 651
- US-A- 3 620 808
- US-A- 3 657 784
- US-A- 3 736 109
- US-A- 3 890 456
- US-A- 4 159 353
- US-A- 4 851 300

## Description

This invention relates to an article for use at high temperatures and in corrosive environments and in particular to a protected article. This invention also relates to a method of coating metallic substrates.

The glass industry has a particular need for materials which have both good stability at high temperatures and good corrosion resistance for the manufacture of apparatus that contacts molten glass. Examples of such apparatus are crucibles, stirrers, crown spinners, thermocouple sheaths, etc. The difficulties encountered with apparatus which either contacts molten glass or the atmosphere above the molten glass are the high temperatures, of the order of 1000°-1600°C, the viscosity and abrasiveness of the molten glass and the reactivity of the glass itself. Molten glass will attack, for example crucibles or containers in which it is held, and this attack is most pronounced at the glass line where the glass and air interface and the surface of the glass contacts the crucible or container wall. With time the glass attacks the wall of the apparatus, eg crucible or container and forms a hollow at the glass line as shown in Figure 1 of the accompanying drawing which depicts a portion of a wall 1 of a crucible containing molten glass 2 with air 3 above glass. At the glass 2-air 3 interface denoted by 4, the wall of the crucible has eroded 5 due to the corrosive effect of the glass. Furthermore as a result of the reactivity of the glass small fragments of the apparatus in contact with glass may break off and contaminate the glass. This is a particular disadvantage when the glass is being used for high quality products such as television tubes which should have no visible defects. The chemical attack by the molten glass may also result in metals or compounds being leached into the glass which results in undesirable discolouration.

Apparatus for use in the glass industry is often fabricated from transition or refractory metals or alloys such as nickel alloys or metals or alloys of molybdenum, tantalum, etc in order to provide apparatus with a reasonable time period in service. Platinum group metals defined as ruthenium, rhodium, palladium, osmium, iridium and platinum or alloys thereof have also been used as the material for such apparatus since these metals and alloys have good corrosion resistance to molten glass and good thermal stability. However, the one major disadvantage with using platinum group metals is the high cost of the material itself. To overcome the disadvantage of having apparatus fabricated solely from platinum group metals and alloys apparatus is made with a metallic substrate that is coated or clad therewith, in particular with platinum. In order to provide effective protection the coating or cladding must be of sufficient thickness to protect the substrate for a service life of eg, 3-6 months. These coatings or claddings provide some protection and enable the service life to be increased. The coating or cladding of platinum however does not prevent the major problem of diffusion of oxidants through to the substrate which results in corrosion of the substrate.

Gas turbine blades operate at high temperatures between 600°C and 1100°C and in corrosive environments. A coating of ceramic applied to the blades provides some protection. However, although the ceramic coating does protect the blades from the high temperatures the ceramic coating suffers considerable corrosion. Another disadvantage is the tendency for spalling to occur with the ceramic coating lifting from the blades and becoming detached.

In FR-A-2084651 (Societe Johnson Matthey & Co Ltd) is disclosed a method of sheathing refractory metal articles with platinum group metals for use at high temperature. The refractory metal core is coated with a barrier layer of magnesia and the so-formed core/barrier unit is sheathed with a platinum group metal or an alloy thereof.

US 3890456 (Dils) discloses a method of coating a gas turbine engine component. A substrate of a superalloy has three layers deposited on it. The first layer is a rare earth and aluminium-containing alloy which is oxidised to increase adherence of the subsequently deposited noble metal second layer. Each layer is sufficiently thin to allow oxygen to diffuse through to the first layer, oxidising it to form a third layer of aluminium oxide.

An object of the present invention is to provide an article with improved corrosion resistance and heat stability which overcomes at least some of the disadvantages of the prior art, especially the problem of diffusion of oxidants through to the substrate.

Accordingly the invention provides an article for use at high temperatures and in corrosive environments comprising a metallic substrate on which is deposited successively,
i) a first coating of one or more metals or alloys,
ii) an optional second coating of a mixture of one or more ceramics and one or more metals or alloys,
iii) a third coating of one or more ceramics, and
iv) a fourth coating of one or more platinum group metals or alloys thereof, the fourth coating being substantially non-porous.

The invention further provides a method of making an article comprising applying, successively, to a metallic substrate a first coating of one or more metals or alloys, an optional second coating of a mixture of one or more ceramics and one or more metals or alloys, a third coating of one or more ceramics and a fourth coating of one or more platinum group metals or alloys thereof, and making the fourth coating substantially non-porous.

The invention further provides the use of an article of the invention in contact with molten glass or the atmosphere above molten glass.

References following to a metal or metals include an alloy or alloys of the metal or metals, unless otherwise indicated.

Preferably the metallic substrate is a metal that has some corrosion resistance and/or thermal stability at high temperatures such as refractory metals, eg nickel, molybdenum, tantalum, niobium or tungsten or an alloy of any of these. Other suitable alloys are high melting point intermetallics such as nickel aluminides, cobalt aluminides, tantalum aluminides, platinum group metal intermetallics etc. The metallic substrate may have a surface oxide layer.

The metal of the first coating is preferably compatible with the ceramic of the second coating such that once the substrate is coated the ceramic is not degraded by the metal reacting with the ceramic. The metal is preferably selected from metals that have one or more of the following characteristics; i) good corrosion resistance and good thermal stability, ii) good ductility and iii) thermal coefficient of expansion intermediate the thermal coefficient of expansion of the metallic substrate and the ceramic of the second coating. Preferably the metal is such that the coating is formed with release of energy, preferably by formation of an intermetallic compound. Suitable metals are nickel-aluminium, nickel-chromium, palladium-aluminium, hafnium-aluminium, titanium, tantalum and palladium. Most preferred is an alloy of nickel 80wt% aluminium 20wt%.

The first coating may be deposited onto the substrate by known methods of application such as thermal spraying and in particular flame or vacuum- or air-plasma spraying.

The second coating comprises a mixture of one or more ceramics and one or more metals. Preferably the ceramic consists essentially of at least one of alumina, magnesia, hafnia, thoria and zirconia. Most preferably the ceramic consists essentially of alumina. Optionally the ceramic may include a minor amount of one or more yttria, silica, titania and calcia. Most preferably the ceramic is of high purity of the order of 99% purity. The metal is preferably the same metal as that of the first coating. Preferably the second coating has a composition in which the proportion of metal to ceramic decreases in gradations from that at the interface adjacent the first coating to that at the interface adjacent the third coating. The second coating may be formed by thermal spraying, for example by vacuum- or air-plasma spraying and in particular the coating may be formed by the deposition of one or more layers. A plurality of layers can be employed to form a step-wise gradation of the metal to ceramic ratio as mentioned above.

The third coating of ceramic preferably consists essentially of alumina. Suitable other materials for the third coating may be magnesia, hafnia, thoria or zirconia or a mixture thereof. Optionally the ceramic may include a minor amount of one or more of yttria, silica, titania and calcia. This coating may be deposited by thermal spraying and in particular by flame- or vacuum- or air-plasma spraying one or more layers.

The fourth coating is substantially non-porous and is chosen from platinum, an alloy of platinum, eg platinum with 5% gold, or zirconia grain stabilised (ZGS) platinum. Other platinum group metals may also be employed. The coating may be deposited for example by flame- or vacuum- or air-plasma spraying, as a powder, or by plating. Preferably the coating is applied by thermal spraying and in particular by flame- or vacuum- or air-plasma spraying. The coating can be made non-porous by after-treatment. The after-treatment may comprise shot peening, melt glazing, hot isostatic pressing (hip) or cold isostatic pressing (cip). The thickness of the fourth coating is typically, between 75 and 200µm; however, there is no upper limit as to how thick the fourth coating may be. Preferably, the thickness of the fourth coating is at least 90µm.

Usually the article consists of the metallic substrate and the four specified coatings. However, in some cases, only the first, third and fourth coatings need be employed.

In a particular embodiment which is not an embodiment of the invention, the article has an additional fifth coating between the third and fourth coatings, the fifth coating being a mixture of one or more ceramics and one or more platinum group metal or silver or gold or alloys thereof. Preferably the ceramic consists essentially of alumina. Other suitable ceramics may be magnesia, hafnia, thoria or zirconia or a mixture thereof. Optionally the ceramic may include a minor amount of one or more of yttria, titania, silica and calcia. Most preferably the ceramic is of high purity, of the order of 99% purity. Preferably the fifth coating has a composition in which the proportion of metal to ceramic increases in gradations from that at the interface with the third coating to that at the interface with the fourth coating. The fifth coating may be formed by thermal spraying, for example by flame- or vacuum- or air-plasma spraying and in particular the coating may be formed by the deposition of one or more layers. A plurality of layers can be employed to form a step-wise gradation of the metal to ceramic ratio as mentioned above.

Figure 2 is a cross-section of an article according to the present invention.

An embodiment of the present invention is shown in Figure 2. A metallic substrate 10 has a first coating 11 of a metal or alloy, a second coating 12 of a mixture of one or more metals and alloys and of at least one ceramic, a third coating 13 of at least one ceramic and a fourth non-porous coating 14 of a platinum group metal or alloy thereof. In the second coating 12 the proportion of metal or alloy to ceramic decreases from the interface with the first coating 11 to the interface with the third coating 13 as schematically depicted with '-' for metal or alloy of the first and second coatings and '+' for the ceramic of the second and third coatings.

The invention will now be described by way of example only.

### COMPARATIVE EXAMPLE

Nicrobell A is the trade name of a Cr/Al/Ti/Y₂O₃/Fe alloy, produced by Nicrobell Pty Ltd.

Nicrobell X is the trade name of a Cr/Si/Mg/Ni alloy produced by Nicrobell Ptv Ltd.

A number of test samples of refractory alloys in the form of tubes were coated with a platinum coating of various thicknesses. The platinum was deposited by means of a fused salt plating bath. One of the samples, Nicrobell A with a platinum coating of 60µm had been subjected to a preoxidation treatment so that the Nicrobell A substrate had a thin oxide layer on to which the platinum was applied. The samples were tested by placing the sample in contact with molten bottle glass at a temperature of 1200°C for a period of time. Each sample was placed with one end in an alumina crucible and bottle glass powder added such that on heating the crucible to a temperature of 1200°C a portion of the sample is in contact with molten glass. At the end of the test the samples were visually examined to see the corrosive effect on the sample by the glass. The results for a 24 hour test are given in Table 1 below. The alloys Nicrobell X and Nicrobell A consist of chromium 20%, aluminium 4.5%, titanium 0.5%, Y₂O₃ 0.5%, remainder iron, and chromium 14.0%, silicon 1.4%, magnesium 0.2% and remainder nickel, the percentages being by weight.

**Table 1**

| Substrate | Pt Coating Thickness µm | |
|---|---|---|
| Nicrobell A | 46 | Ni diffused through Pt coating. |
| Nicrobell A | 60 | Pt coating lifted off by diffusion. |
| Nicrobell X | 72 | Fe diffused through Pt coating. |
| | | Al reaction with Pt. |

The results of the tests given in Table 1 above show that a single coating of platinum between 46µm and 72µm onto a metallic substrate does not prevent corrosion by molten glass.

### Examples 1-12

A number of tubes were fabricated from a commercial nickel-based alloy, nickel 75wt%, chromium 25wt%. A first coating of nickel was applied thereto followed by a second coating of nickel and alumina formed by three layers having the Ni:Al₂O₃ proportions 1:1, 1:3 and 1:9 respectively. The third coating of alumina was applied as one or more layers. The first, second and third coatings were applied using vacuum-plasma spraying. Examples 1 to 4 were provided with a conductive surface by sputter deposition of 0.2µm films of platinum in preparation for a fourth coating of platinum deposited by electro-deposition from a bath of composition disclosed in Example 1 of EP 0358375 A with 5-5.5g of platinum per litre. Examples 1, 2 and 3 which are not embodiments of the invention, had an additional top coating of 0.2µm of gold deposited by sputtering. The fourth coating of Examples 5 to 8 was applied by a fused salt process. Examples 9-12 had the fourth coating deposited by flame-spraying. The Examples were tested for 300 hours by contacting with molten glass as described in Comparative Example A and the results are given in Tables 2, 3 and 4. AGL, GL and BGL denote 'Above Glass Line', 'Glass Line' and 'Below Glass Line'.

### Conclusion

Examples 1-12 demonstrate that the four-layer coating system is capable of protecting base metal substrate. However, very thin fourth coatings were largely ineffective below the glass line.

### Comparative Examples B and C

### Example 13

Example 13 comprised a closed end tube of Nicrobell A with a first coating of Ni 96wt% Al 4wt%, a second coating of nickel and alumina formed by three layers having Ni:Al₂O₃ proportions of 1:1, 1:3 and 1:9, a third coating of alumina and a fourth coating of platinum of thickness 6.1µm. Comparative Example B was a tube of Nicrobell A with a first coating of Ni 96wt% Al 4wt%, a second coating of alumina graduated from low to high density and a third coating of platinum of thickness 4.8µm. For Comparative Example C a Nicrobell A closed end tube was coated with a first coating of alumina graduated from low to high density and a second coating of platinum, thickness 5.5µm. The coatings of Ni 96wt% Al 4wt%, alumina and nickel and alumina were applied by vacuum plasma spraying. After the surface was rendered conductive by sputter-deposition of a sub-micron film of platinum, the fourth coatings of platinum were deposited by electro-deposition from a bath of composition as described in Example 1 of EP 0358375 A with 5-5.5g of platinum per litre. These examples were tested for 300 hours by contacting the tubes with molten glass as described above in Comparative Example A and the results are given in Table 5 below. The Nicrobell A alloy has the composition chromium 14wt%, silicon 1.4wt%, magnesium 0.25wt% and remainder nickel.

The results given in Table 5 above indicate that to provide articles which can be used at high temperatures and in corrosive environments four different specific coatings are required. While in each case the Pt layer was too thin to be effective, and flaked off, the third layer was significantly more intact in the four coating Example as compared with the three coating Comparative Example.

### Examples 14-21

Examples 14 to 21 employed closed end tubes of Nicrobell A or Nicrobell C as substrates. Nicrobell C is the trade name of an alloy of composition chromium 23.9wt%, silicon 1.75wt%, magnesium 0.15wt%, niobium 0.49wt% and remainder nickel, produced by Nicrobell Pty Ltd. The composition of the first coating for these examples was nickel 80wt%, aluminium 20wt%. The second coating of Ni 80wt% Al 20wt% and alumina was deposited as three layers with various proportions of Ni 80wt%, Al 20wt%: alumina. Details are given in Table 6 below. Between 4 and 30 layers of alumina were deposited to form the third coating. The first, second and third coatings were deposited by vacuum plasma spraying. The fourth layer of platinum was formed by flame-spraying followed by an after treatment of shot-peening to ensure the fourth coating was substantially non-porous.

The examples were tested by contacting them with molten glass for 300 hours as described above. The results are given in Table 6 below.

Example 16 was not tested as cracks appeared prior to platinum coating. This was probably due to the thickness of the third coating which was formed from thirty layers of alumina. The results obtained for Examples 14, 15 and 20 with a second coating having the amount of metal decreasing from the interface with the first coating to the interface with the third coating are better than for Examples 17, 18, 19 and 21 where the proportion of metal to ceramic was the same through the thickness of the second coating.

### Comparative Example D

### Examples 22-24

Comparative Example D and Examples 22-24 employed substrates of Nicrobell C. The first coat for each was nickel 80wt%, aluminium 20wt%. Examples 22-24 employed second coats of Ni 80wt% Al 20wt% and alumina deposited in the ratios 1:1, 1:3 and 1:9, and third coats, of 8 layers of either alumina or zirconia. Comparative Example D omitted coats 2 and 3. The first, second and third coats were deposited by vacuum- plasma spraying. The fourth layer of Pt or Pt/5wt% Au was flame-sprayed followed by shot peening to ensure that the fourth layer be substantially non-porous.

The examples were tested in molten glass at 1200°C for 400 hours, the results are given below.

The results obtained for Examples 22, 23 and 24 show that the coatings have protected the substrates from molten glass attack, the thicker the platinum group metals (PGM) layer (Example 23) the better the degree of protection. A thicker layer of PGM gives ore ductility. Adequate PGM coating ductility is essential to promote protection.

### Examples 26-28

Examples 26-28 are components to be used in temperature measurement. They were manufactured using Nicrobell C substrates, for trials in an industrial glass bottle manufacturing plant. The coating system applied was identical to that for Example 23. The example components were placed in a forehearth containing flowing molten flint glass at a temperature which ranged from 1130-1160°C for varying times. The details are given below.

| ID | Substrate | 1st coat | 2nd 1st:3rd1:1,1:3, 1:9 | 3rd no of layers Al₂O₃ | 4th PGM thickness | Duration of test | Typical temperature °C |
|---|---|---|---|---|---|---|---|
| 26 | Nicrobell C | Ni20%Al | 1/1/1 | 8 | Pt 169µm | 24 hrs | 1137°C |
| 27 | Nicrobell C | Ni20%Al | 1/1/1 | 8 | Pt 171µm | 100 hrs | 1160°C |
| 28 | Nicrobell C | Ni20%Al | 1/1/1 | 8 | Pt 174µm | 1000 hrs | 1160°C |

Results - Coating condition after test.

After testing all Examples (26-28) were completely intact, no corrosion had occurred nor cracking on cooling. The example components had been removed from the molten glass before cooling unlike the laboratory tests where the examples cooled in situ. The glass below the glass line had not adhered to the samples evenly. Some areas had been left completely free of glass. On cooling, particularly Example 28, the attatched glass cracked and fell away from the metal surface. The coating was concluded to have 'nonstick' characteristics. This is an added advantage reducing any cross-contamination and aiding recycling and examination of the components.

### Example 29-32

Examples 29-32 employed substrates of Nicrobell C. The first coat was nickle 80wt%, aluminium 20wt%, the second coats were Ni 80wt%, Al 20wt% and alumina deposited in the ratios 1:1, 1:3 and 1:9. The third coats were 8 layers of alumina. The first, second, and third coats were deposited by vacuum plasma spraying. The fourth layers, of Pt or Pt/5wt% Au were flame sprayed, with this coating in some cases being completed by deposition of ZGS Pt or Pt 5wt%Au. This was followed by shot peening to ensure that the outer metal coating be substantially non-porous.

The examples were tested in molten glass in the laboratory at 1200°C for 400 hours, the results are given below.

The results for Examples 29-32 indicate that a molten glass resistant coating can be produced from ZGS Pt. To achieve protection with Pt 5wt%Au a considerably thicker metal coating is required than with Pt alone.

### Examples 33-38

The substrates employed in Examples 33-38 were selected from Nicrobell C and MA956 alloy closed end tubes. MA956 is the trade name of an alloy of composition Fe 74wt%, Cr 20wt%, Al 4.5wt%, Ti 0.5wt% and Y₂O₃ 0.5wt% produced by Inco Alloys Ltd. The first coat was nickel 80wt%, aluminium 20wt% or nickel 95.5wt%, aluminium 4.5wt%, deposited by vacuum-plasma spraying (VPS) and air-plasma spraying (APS) respectively. For the APS samples in this instance the second coating was absent, however, for Example 37 the coating system was as in Examples 26-28. The third layer was of alumina of thicknesses 120-245µm. The fourth layer of Pt was deposited and processed as per Examples 26-28. The examples were tested in molten glass for 200 hrs at 1200°C, details presented below.

| DURATION OF TEST -200 Hours | | | | | | |
|---|---|---|---|---|---|---|
| Coatings | | | | | | |
| ID | Substrate | Spraying Technique | 1st coat | 2nd Ni:Al₂O₃ 1:1, 1:3, 1:9 | 3rd No. of Al₂O₃ | 4th PGM thickness |
| 33 | Nicrobell C | APS | Ni4.5%Al | - | 135µm | Pt 148µm |
| 34 | Nicrobell C | APS | Ni4.5%Al | - | 245µm | Pt 159µm |
| 35 | MA956 | VPS | Ni20%Al | 1/1/1 | 160µm | Pt 138µm |
| 36 | MA956 | VPS | Ni20%Al | - | 160µm | Pt 160µm |
| 37 | MA956 | APS | Ni4.5%Al | - | 220µm | Pt 164µm |
| 38 | MA956 | APS | Ni4.5%Al | - | 120µm | Pt 166µm |

The thickness of the ceramic layers that have been quoted in all the previous examples are in layers. An approximate converation factor is that one layer is equal to 20µm.

### Results - Coating condition after test

33.
   - AGL: Ni/Cr diffusion present- no cracks
   - GL: Diffusion but coating intact
   - BGL: coating OK
   Glass colour - green, substrate substantially protected.
34.
   - AGL: Very slight Ni/Cr diffusion
   - GL: good coating
   - BGL: good coating
   Glass colour - pale green, substrate protected.
35.
   - AGL: no observable effect
   - GL: no observable effect
   - BGL: no observable effect
   Glass colour - pale green, substrate protected.
36.
   - AGL: no observable effect
   - GL: no observable effect
   - BGL: no observable effect
   Glass colour - pale green, substrate protected.
37.
   - AGL: localized failure with breakaway oxidation
   - GL: coating OK, no diffusion
   - BGL: coating OK, no diffusion
   Glass colour - pale green, substrate essentially protected.
38.
   - AGL: coating disrupted in localised zones
   - GL: coating ok
   - BGL: coating ok
   Glass colour - pale green, substrate essentially protected.

For the short duration no noticeable difference occured between the VPS examples without or with the barrier layer. The APS examples indicate that as long as sufficient thickness of barrier layer is laid down, to offset the effect of increased porosity, protection is given. Examples 35-36 indicate, iron based alloys, such as the corrosion resistant alloy MA956, can be given additonal protection for service in molten glass enviroment by application of a coating system according to this invention.

## Claims

1. An article for use in high temperature corrosive environments comprising a metallic substrate on which is deposited successively:
I) a first coating of one or more metals or alloys,
ii) an optional second coating of a mixture of one or more ceramics and one or more metals or alloys,
iii) a third coating of one or more ceramics, and
iv) a fourth coating of one or more platinum group metals or alloys thereof, the fourth coating being substantially non-porous.

2. An article according to claim 1 wherein the metallic substrate has deposited all four said coatings.

3. An article according to claim 1 or 2 wherein the first coating is of a metal or alloy selected from nickel-aluminium, nickel-chromium, palladium-aluminium, hafnium-aluminium, titanium, tantalum and palladium.

4. An article according to claim 3 wherein the first coating is of an alloy of nickel 80wt% aluminium 20wt%.

5. An article according to any preceding claim wherein the ceramic of the second and third coatings is alumina.

6. An article according to claim 5 wherein the ceramic is of purity 99%.

7. An article according to any preceding claim wherein the second coating has a composition in which the proportion of metal to ceramic decreases from the interface adjacent the second coating.

8. An article according to any preceding claim wherein the fourth coating is of platinum or an alloy of platinum.

9. An article according to any preceding claim wherein the fourth coating is of platinum.

10. Use of an article according to any preceding claim, in contact with molten glass or the atmosphere above molten glass.

11. A method of making an article claimed in any one of claims 1-9 comprising applying, successively, to a metallic substrate a first coating of one or more metals or alloys, an optional second coating of a mixture of one or more ceramics and one or more metals or alloys, a third coating of one or more ceramics and a fourth coating of one or more platinum group metals or alloys thereof, and making the fourth coating substantially non-porous.

## Patentansprüche

1. Gegenstand zur Verwendung in einer korrosiven Umgebung mit höherer Temperatur umfassend ein Metallsubstrat, auf dem nacheinander abgeschieden wurden:
i) eine erste Beschichtung aus einem oder mehreren Metallen oder Legierungen,
ii) gegebenenfalls eine zweite Beschichtung aus einer Mischung von einer oder mehreren Keramiken und einem oder mehreren Metallen oder Legierungen,
iii) eine dritte Beschichtung aus einer oder mehreren Keramiken und
iv) eine vierte Beschichtung aus einem oder mehreren Metallen der Platingruppe oder Legierungen davon, wobei die vierte Beschichtung im wesentlichen nicht porös ist.

2. Gegenstand nach Anspruch 1, worin auf dem Metallsubstrat alle vier Beschichtungen abgeschieden wurden.

3. Gegenstand nach Anspruch 1 oder 2, worin die erste Beschichtung aus einem Metall oder einer Legierung ist, die ausgewählt sind aus Nickel-Aluminium, Nickel-Chrom, Palladium-Aluminium, Hafnium-Aluminium, Titan, Tantal und Palladium.

4. Gegenstand nach Anspruch 3, worin die erste Beschichtung eine Legierung aus 80 Gew.-% Nickel, 20 Gew.-% Aluminium ist.

5. Gegenstand nach einem der vorhergehenden Ansprüche, worin die Keramik der zweiten und dritten Beschichtung Aluminiumoxid ist

6. Gegenstand nach Anspruch 5, worin die Keramik eine Reinheit von 99% hat.

7. Gegenstand nach einem der vorhergehenden Ansprüche, worin die zweite Beschichtung eine Zusammensetzung hat, in der das Verhältnis von Metall zu Keramik von der der zweiten Beschichtung benachbarten Grenzfläche hin abnimmt.

8. Gegenstand nach einem der vorhergehenden Ansprüche, worin die vierte Beschichtung aus Platin oder einer Platinlegierung ist.

9. Gegenstand nach einem der vorhergehenden Ansprüche, worin die vierte Beschichtung aus Platin ist.

10. Verwendung eines Gegenstands nach einem der vorhergehenden Ansprüche für den Kontakt mit geschmolzenem Glas oder mit der Atmosphäre oberhalb des geschmolzenen Glases.

11. Verfahren zur Herstellung eines Gegenstands nach einem der Ansprüche 1 bis 9 umfassend, daß man aufeinanderfolgend auf ein Metallsubstrat eine erste Beschichtung aus einem oder mehreren Metallen oder Legierungen, gegebenenfalls eine zweite Beschichtung aus einer Mischung aus einer oder mehreren Keramiken und einem oder mehreren Metallen oder Legierungen, eine dritte Beschichtung aus einer oder mehreren Keramiken und eine vierte Beschichtung aus einem oder mehreren Metallen der Platingruppe oder Legierungen davon aufträgt und die vierte Beschichtung im wesentlichen nicht-porös macht.

## Revendications

1. Objet destiné à servir dans des environnements corrosifs où règne une température élevée, cet objet comprenant un substrat métallique sur lequel est déposé successivement :
i) un premier revêtement, formé d'un ou plusieurs métaux ou alliages,
ii) un second revêtement, facultatif formé d'un mélange d'une ou plusieurs matières céramiques et d'un ou plusieurs métaux ou alliages,
iii) un troisième revêtement, formé d'une ou plusieurs matières céramiques, et
iv) un quatrième revêtement, formé d'un ou plusieurs métaux ou alliages du groupe ou de la famille du platine, le quatrième revêtement étant essentiellement non poreux.

2. Objet selon la revendication 1, dans lequel le substrat métallique comporte, déposés, l'ensemble des quatre dits revêtements.

3. Objet selon la revendication 1 ou 2, dans lequel le premier revêtement est en un métal ou alliage choisi parmi du nickel-aluminium, du nickel-chrome, du palladium-aluminium, du hafnium-aluminium, du titane, du tantale et du palladium.

4. Objet selon la revendication 3, dans lequel le premier revêtement est en un alliage formé de 80 % en poids de nickel et de 20 % en poids d'aluminium.

5. Objet selon l'une quelconque des revendications précédentes, dans lequel la matière céramique des second et troisième revêtements est de l'alumine.

6. Objet selon la revendication 5, dans lequel la matière céramique a une pureté de 99 %.

7. Objet selon l'une quelconque des revendications précédentes, dans lequel le second revêtement a une composition dans laquelle le rapport ou proportion du métal à la matière céramique diminue depuis l'interface voisine du second revêtement.

8. Objet selon l'une quelconque des revendications précédentes, dans lequel le quatrième revêtement est en platine ou en un alliage de platine.

9. Objet selon l'une quelconque des revendications précédentes, dans lequel le quatrième revêtement est en platine.

10. Utilisation d'un objet selon l'une quelconque des revendications précédentes, en contact avec du verre fondu ou avec l'atmosphère située au-dessus de verre fondu.

11. Procédé pour produire un objet tel que revendiqué dans l'une quelconque des revendications 1 à 9, ce procédé comprenant l'application, successivement, à un substrat métallique d'un premier revêtement formé d'un ou plusieurs métaux ou alliages, d'un second revêtement facultatif formé d'un mélange d'une ou plusieurs matières céramiques et d'un ou plusieurs métaux ou alliages, d'un troisième revêtement formé d'une ou plusieurs matières céramiques et d'un quatrième revêtement formé d'un ou plusieurs métaux ou alliages de métaux du groupe ou de la famille du platine, et la réalisation du quatrième revêtement en un état essentiellement non poreux.
